

Oct. 9, 1973

HIROSHI HIRANO ETAL

3,764,407

METHOD FOR PRODUCING A MONO-DIRECTIONAL SILICON STEEL SHEET

Filed Feb. 9, 1972

3 Sheets-Sheet 1

*FIG. 1*



*FIG. 2*



Oct. 9, 1973

HIROSHI HIRANO ETAL

3,764,407

METHOD FOR PRODUCING A MONO-DIRECTIONAL SILICON STEEL SHEET

Filed Feb. 9, 1972

3 Sheets-Sheet 2

FIG. 3



FIG. 4



Oct. 9, 1973

HIROSHI HIRANO ETAL

3,764,407

METHOD FOR PRODUCING A MONO-DIRECTIONAL SILICON STEEL SHEET

Filed Feb. 9, 1972

3 Sheets-Sheet 3

FIG. 5

No. C      No. 126      No. 128      No. 133      No. 136



FIG. 6

No. C      No. 126      No. 128      No. 133      No. 136



1

3,764,407

**METHOD FOR PRODUCING A MONO-DIRECTIONAL SILICON STEEL SHEET**

Hiroshi Hirano, Nishinomiya, Kiyoshi Yoshida, Kakogawa, and Nobutaro Kusuoka, Kobe, Japan, assignors to Kobe Steel, Ltd., Kobe-shi, Japan

Continuation-in-part of abandoned application Ser. No. 817,485, Apr. 18, 1969. This application Feb. 9, 1972, Ser. No. 224,853

Claims priority, application Japan, Apr. 24, 1968,  
43/27,582

Int. Cl. H01f 1/04

U.S. Cl. 148—112

2 Claims

**ABSTRACT OF THE DISCLOSURE**

A mono-directional silicon steel sheet having excellent electromagnetic characteristic is produced by using a silicon steel containing 2-4% of Si and small amount of Al, Ti, Zr or Ta or at least two of Al, Ti, Zr and Ta and subjecting the steel sheet to nitriding treatment at 450°-750° C. before a final annealing.

This is a continuation-in-part of our application, Ser. No. 817,485 filed on Apr. 18, 1969, now abandoned.

This invention relates to a method for producing a mono-directional silicon steel sheet having excellent electromagnetic characteristics. The term "sheet" herein used also includes a strip.

The mono-directional silicon steel sheet used for core material of a transformer, etc. is polycrystalline. When each crystal grain which is a constructive element of the silicon steel sheet is oriented in the direction of (110) <100>, a soft electromagnetic material can be produced having a low iron loss and a high magnetic flux density by passing magnetic flux in the direction of <100>. Such electromagnetic material has been produced on an industrial scale. However, in the industrial production of said material, the establishment of a technique for obtaining a stable secondary recrystallization structure has been a problem and many proposals have been made as a possible solution. Most of the conventional methods for producing a mono-directional silicon steel sheet, with some exceptions, have in common the utilization of a dispersed fine precipitate to prevent normal grain growth of primary recrystallization. However, the control of the precipitation state of the dispersed fine precipitate must be monitored through the entire production run beginning with the initial chemical composition of an ingot, heating of the ingot, hot rolling, water cooling after hot rolling, coiling temperature of steel strip and the subsequent cold rolling, annealing, etc. As a result, unusual and careful quality control must be used to produce a mono-directional silicon steel sheet with good reproducibility and in a high yield.

As is well known, for example, MnS is widely used to restrict normal grain growth and to obtain complete secondary recrystallization. However, in the event of MnS, the content of Mn and S must precisely be controlled to ensure solution of MnS during heating of the slab before hot rolling to hot rolled steel band.

In addition, the precise controls of the finishing temperature of hot rolling and the coiling temperature are required to get finely and uniformly dispersed MnS particles, and also the ingot size of 3 percent silicon steel must be limited to around 7 tons to minimize sulphur segregation.

It is therefore an object of this invention to provide a method for producing a highly stable mono-directional silicon steel sheet with good reproducibility by subjecting a silicon steel, containing 2-4% of Si and the balance of

2

iron including inevitable impurities, to which a small amount of one element selected from the group consisting of Al, Ti, Zr and Ta or two or more of elements selected from the group consisting of Al, Ti, Zr and Ta are added as a nitride producing element, to hot rolling, and cold rolling to the given thickness, decarburization, etc. in accordance with the conventional methods, to nitriding treatment for nitriding said nitride producing elements and to the final annealing treatment to orient the crystal direction to the direction of (110) <100> after the final annealing.

According to this invention, elements, Al, Ti, Zr and Ta added to the silicon steel are nitrided by a nitriding treatment for attaining secondary recrystallization before the final annealing to produce nitrides of said elements and said nitrides act effectively as dispersed precipitate for preventing the normal grain growth of primary recrystallization. These elements also ensure the production of a mono-directional silicon steel sheet having secondary recrystallization structure. Adding nitride producing elements to silicon steel and nitriding said elements with a suitable nitriding treatment immediately before the final annealing to produce the nitrides simplify the practice of our process since the extensive monitoring of the several stages is unnecessary to our process.

A characteristic of this invention is the addition of said nitride producing elements to the silicon steel used. When said element is added alone, Al should be added within the range of 0.01-0.07% by weight, Ti within 0.01-0.2% by weight, Zr within 0.01-0.3% by weight and Ta within 0.05-0.5% by weight. When two or more of them are added, Ti, Zr, Ta and Al are added within the ranges as mentioned above, but the total amount should not exceed 0.5%.

The reasons for the restrictions of the amounts of the nitride producing elements as mentioned above are as follows: (i) when the amounts are less than their lower limits, the amount of nitride produced is insufficient to prevent the normal grain growth of the primary recrystallization grains and no growth of stable secondary recrystallization is observed and (ii) when the amounts are more than the upper limits, excess nitrides are precipitated to prevent the growth of the secondary recrystallization.

Si is added primarily for improving magnetic characteristic and is added in an amount of 2-4% in view of industrial production. Furthermore, the silicon steel should contain carbon in an amount of 0.01-0.10% for the following reasons. Since carbon has a bad effect on magnetic property, the amount should be as small as possible. However, when carbon content is less than 0.01 in the production of steel ingot, insufficient deoxidation of the steel takes place. Since steel containing a large amount of oxygen deteriorates the magnetic property of the steel, the lower limit of carbon is specified as 0.01%. When the amount of carbon is more than 0.1%, decarburization becomes difficult and time consuming and further the texture of the sheet upon cold rolling and annealing is also affected. Therefore, the carbon content is restricted to 0.01-0.10%.

Another characteristic of this invention is that a silicon steel sheet containing said nitride producing elements is subjected to nitriding treatment immediately before final annealing. Said nitriding treatment can be attained merely by heating the silicon steel sheet in an atmosphere of pure nitrogen gas, hydrogen-nitrogen mixture gas capable of nitriding or ammonia decomposition gas from liquid ammonia. The heating temperature in said nitriding treatment must be between from 450° to 750° C. for industrial production. This is because the silicon steel sheet must be heated at a temperature as low as possible in order to avoid softening and coil set of the sheet due to high tem-

perature. As is known, the softening and coil set are affected by thickness and width of the sheet as well as nitriding temperature. Hence, since the nitriding treatment is carried out after the completion of the primary recrystallization by decarburization treatment in a continuous furnace, the nitriding temperature within the range of 450° to 750° C. can be determined with due regard to coil set due to coil softening, and by criteria known to those skilled in the art, the most economical temperature within said range can accordingly be optionally selected.

The heating temperature in the nitriding treatment, which depends upon, nitrogen partial pressure and the kind and amount of nitride producing elements contained in the steel, is about 2-20 hours within which time secondary recrystallization can be achieved.

Conditions other than those above mentioned which have not been specified as a characteristic of this invention may be suitably chosen and employed. For example, for rolling the silicon steel to a desired thickness, the steel is hot rolled, thereafter is subjected to pickling and annealing, and then is subjected to cold rolling which includes twice and single cold rolling methods. According to the single cold rolling method, a steel sheet of 1.5-2.5 mm. in thickness is cold rolled with a reduction rate of 70-90% to a desired thickness and is subjected to nitriding treatment after decarburization step. According to the double cold rolling method, a steel sheet of 2-3 mm. in thickness is first subjected to a rolling with a reduction rate of 50-80%, then to decarburization treatment at 700°-900° C., thereafter to the second cold rolling with a reduction rate of 40-60%, again to decarburization treatment, and then to nitriding treatment.

The nitride forming elements in this invention must be classified into two groups from the thermodynamic point of view, that is, the groups of Ti and Zr, and Al and Ta. Titanium and zirconium form more stable compounds with nitrogen than any other commonly used alloying elements, that is, titanium and zirconium nitrides are much more stable than aluminum and tantalum nitrides.

The thermodynamic data concerning the equilibrium between Ti and N or Zr and N in ferrite, particularly in 3 percent silicon steel are still lacking.

In order to attempt a qualitative estimation of the behaviors of these nitride forming elements in 3 percent silicon steel, the thermodynamic relationships in gamma or alpha iron shown below are taken and the quantities of nitrogen in solution or as compound with each nitride forming element are calculated under the given conditions.

The empirical formula and the results of calculation are as follows.

TABLE 1

| Temp.<br>(° C.) | Element | Element in solution  | $\Sigma N = 0.009\%$ | $\Sigma N = 0.009\%$ |
|-----------------|---------|----------------------|----------------------|----------------------|
|                 |         | Element as compound  | $\Sigma Ti = 0.07\%$ | $\Sigma Ti = 0.03\%$ |
| 5               | N       | {N in solution.....  | 0.0001               | 0.0014               |
|                 |         | {N as TiN.....       | 0.0089               | 0.0076               |
|                 | Ti      | {Ti in solution..... | 0.0396               | 0.0039               |
|                 |         | {Ti as TiN.....      | 0.0304               | 0.0261               |
| 10              | N       | {N in solution.....  | 0.0003               |                      |
|                 |         | {N as TiN.....       | 0.0009               | 0.0087               |
|                 | Ti      | {Ti in solution..... | 0.0391               | 0.0003               |
|                 |         | {Ti as TiN.....      | 0.0309               | 0.0297               |
| 900             | N       | {N in solution.....  | 0.0009               | 0.0003               |
|                 |         | {N as TiN.....       | 0.0391               | 0.0087               |
|                 | Ti      | {Ti in solution..... | 0.0309               |                      |
|                 |         | {Ti as TiN.....      | 0.0309               | 0.03                 |

15 Fe( $\gamma$ )-Zr-N

$$\log [\text{percent Zr}] [\text{percent N}] = -\frac{16,600}{T} + 4.79$$

TABLE 2

| Temp.<br>(° C.) | Element | Element in solution  | $\Sigma N = 0.009\%$ | $\Sigma N = 0.009\%$ |
|-----------------|---------|----------------------|----------------------|----------------------|
|                 |         | Element as compound  | $\Sigma Zr = 0.08\%$ | $\Sigma Zr = 0.03\%$ |
| 25              | N       | {N in solution.....  | 0.0002               | 0.0045               |
|                 |         | {N as ZrN.....       | 0.0088               | 0.0045               |
|                 | Zr      | {Zr in solution..... | 0.0226               | 0.0008               |
|                 |         | {Zr as ZrN.....      | 0.0574               | 0.0292               |
| 30              | N       | {N in solution.....  | 0.0009               | 0.0044               |
|                 |         | {N as ZrN.....       | 0.0215               | 0.0001               |
|                 | Zr      | {Zr as ZrN.....      | 0.0585               | 0.030                |
|                 |         | {Zr in solution..... | 0.009                |                      |

Fe( $\gamma$ )-Ta-N

$$\log [\text{percent Ta}] [\text{percent N}] = -\frac{12,800}{T} + 6.08$$

TABLE 3

| Temp. (° C.) | Element | Element in solution  | $\Sigma N = 0.009\%$ | $\Sigma N = 0.009\%$ |
|--------------|---------|----------------------|----------------------|----------------------|
|              |         | Element as compound  | $\Sigma Ta = 0.2\%$  | $\Sigma Ta = 0.2\%$  |
| 45           | N       | {N in solution.....  | 0.0007               |                      |
|              |         | {N as TaN.....       | 0.002                |                      |
|              | Ta      | {Ta in solution..... | 0.17                 | 0.028                |
|              |         | {Ta as TaN.....      | 0.0042               |                      |
| 50           | N       | {N in solution.....  | 0.0048               |                      |
|              |         | {N as TaN.....       | 0.1374               | 0.0626               |
|              | Ta      | {Ta in solution..... | 0.0002               |                      |
|              |         | {Ta as TaN.....      | 0.0088               |                      |

50 Fe( $\gamma$ )-Al-N

$$\log [\text{percent Al}] [\text{percent N}] = -\frac{7400}{T} + 1.95$$

TABLE 4

| Temperature (° C.) | Element | Element in solution  | $\Sigma N = 0.015\%$ |                      | $\Sigma N = 0.009\%$ |                      |
|--------------------|---------|----------------------|----------------------|----------------------|----------------------|----------------------|
|                    |         | Element as compound  | $\Sigma Al = 0.05\%$ | $\Sigma Al = 0.03\%$ | $\Sigma Al = 0.05\%$ | $\Sigma Al = 0.03\%$ |
| 1,350              | N       | {N in solution.....  |                      |                      |                      |                      |
|                    |         | {N as AlN.....       |                      |                      |                      |                      |
|                    | Al      | {Al in solution..... |                      |                      |                      |                      |
|                    |         | {Al as AlN.....      |                      |                      |                      |                      |
| 1,100              | N       | {N in solution.....  | 0.0093               | 0.0135               | 0.0077               |                      |
|                    |         | {N as AlN.....       | 0.0057               | 0.0015               | 0.0013               |                      |
|                    | Al      | {Al in solution..... | 0.0390               | 0.0270               | 0.0474               |                      |
|                    |         | {Al as AlN.....      | 0.0110               | 0.0030               | 0.0026               |                      |
| 900                | N       | {N in solution.....  | 0.0018               | 0.0045               | 0.0013               | 0.0025               |
|                    |         | {N as AlN.....       | 0.0132               | 0.0105               | 0.0078               | 0.0065               |
|                    | Al      | {Al in solution..... | 0.0245               | 0.0097               | 0.0351               | 0.0175               |
|                    |         | {Al as AlN.....      | 0.0265               | 0.0203               | 0.0150               | 0.0125               |

Fe( $\gamma$ )-Ti-N

$$\log [\text{percent Ti}] [\text{percent N}] = -\frac{16,200}{T} + 4.72$$

Fe( $\alpha$ )-Al-N

$$\log [\text{percent Al}] [\text{percent N}] = -\frac{8300}{T} + 1.69$$

TABLE 5

| Temperature (° C.) | Element | Element in solution    | $\Sigma N = 0.015\%$ |                      | $\Sigma N = 0.009\%$ |                      |
|--------------------|---------|------------------------|----------------------|----------------------|----------------------|----------------------|
|                    |         | Element as compound    | $\Sigma Al = 0.05\%$ | $\Sigma Al = 0.03\%$ | $\Sigma Al = 0.05\%$ | $\Sigma Al = 0.03\%$ |
| 900                | N       | { N in solution -----  | 0.0002               | 0.0012               | 0.0001               | 0.0003               |
|                    |         | { N as AlN -----       | 0.0148               | 0.0138               | 0.0089               | 0.0087               |
|                    | Al      | { Al in solution ----- | 0.0214               | 0.0034               | 0.0329               | 0.0132               |
|                    |         | { Al as AlN -----      | 0.0286               | 0.0266               | 0.0171               | 0.0168               |
| 800                | N       | { N in solution -----  | 0.0004               | 0.0005               | 0.00003              | 0.00007              |
|                    |         | { N as AlN -----       | 0.0150               | 0.0145               | 0.0090               | 0.0089               |
|                    | Al      | { Al in solution ----- | 0.0212               | 0.0020               | 0.0327               | 0.0128               |
|                    |         | { Al as AlN -----      | 0.0288               | 0.0280               | 0.0173               | 0.0172               |
| 700                | N       | { N in solution -----  | 0.0001               | -----                | 0.00001              | -----                |
|                    |         | { N as AlN -----       | 0.0150               | 0.0149               | 0.0090               | 0.0096               |
|                    | Al      | { Al in solution ----- | 0.0211               | 0.0013               | 0.0327               | 0.0127               |
|                    |         | { Al as AlN -----      | 0.0290               | 0.0287               | 0.0173               | 0.0173               |

According to the results of the calculation shown above, the following conclusions are obtained.

(1)  $Fe\text{-Ti-N}$

As is clearly shown in Table 1, most of the nitrogen is fixed as TiN at 1350° C. when N content is 0.009 percent and Ti content is 0.03 percent.

It seems that the size of titanium nitrides formed in molten steel are generally quite large and they are distributed coarsely in solidified steel. Such kinds of titanium nitrides, of course, will, to some extent restrict grain boundary migration, but entire prevention of normal grain growth is impossible.

FIG. 1 is a photograph ( $\times 1,500$ ) showing an example of a large titanium nitride particle which is seemed to be formed in the molten steel, and the effect of the restriction of grain boundary migration.

If the contents of Ti and N in steel are kept at a constant value and the size of titanium nitrides are quite large as shown in FIG. 1, the total number of titanium nitrides become small. In the consequence, absolute prevention of normal grain growth is impossible and complete secondary recrystallization cannot be obtained. In addition, in the event of titanium nitrides, the control of the size and distribution of such nitrides by heat treatment is virtually impossible. This is clearly shown in Table 1.

Accordingly in this invention, only titanium is added to the original melt to the substantial exclusion of nitrogen, the latter if present being contained in the melt as an incidental impurity.

The material mentioned above was processed following the process shown in examples.

FIG. 2 is a photograph ( $\times 1,500$ ) showing the finely dispersed titanium nitrides formed by nitriding treatment prior to final annealing for secondary recrystallization. It is clearly shown that in the case of a strong nitride forming element like titanium, nitriding at low temperature such as 750° C. is the most excellent means to get finely dispersed titanium nitrides. The size of titanium nitrides shown in FIG. 2 is about 70 Å. in average and much smaller than the one shown in FIG. 1.

The is one of the characteristics of this invention.

(2)  $Fe(\gamma)\text{-Zr-N}$

Zirconium is thermodynamically strong nitride forming element next to titanium.

Accordingly the behavior of ZrN is similar to the one of TiN. It is observed from Table 2 that a part of ZrN goes into solution at a temperature of from about 1100° C. to 1350° C. when the contents of Zr and N are 0.03% and 0.009%, respectively. It is also observed from Table 1 that only minor amount of TiN, on the contrary to the case of ZrN, goes into solution.

This is a marked difference between both nitride forming elements.

According to Table 2, when the content of Zr is 0.03%, about half of the total nitrogen goes into solution at 1350° C., but when the content of Zr is 0.08% most of the nitrogen remains still unsolved. It is, therefore, im-

possible to control the size and distribution of zirconium nitrides by successive treatments such as slab heating, hot rolling and the control of coiling temperature.

The formation of zirconium nitrides by nitriding process prior to final annealing for secondary recrystallization is also a quite effective method to obtain finely dispersed zirconium nitrides.

(3)  $Fe(\gamma)\text{-Ta-N}$

As is shown in Table 3, most of the tantalum nitrides go into solution at 1350° C. It is, therefore, possible to control their size and distribution by successive treatments after slabbing. Accordingly, it is also possible to control the size and distribution of the tantalum nitrides by adding nitrogen to an original melt and subjecting it to subsequent heat treatment. However, said control by the heat treatment process requires severe limitations of temperature through the rolling, decarburization and denitridification steps. Therefore, it is very difficult to obtain products having stable properties in the industrial scale production.

(4)  $Fe(\gamma)\text{-Al-N}$  and  $Fe(\alpha)\text{-Al-N}$

As is shown in Tables 4 and 5, the behavior of the aluminum nitrides closely resembles to that of tantalum nitrides. It is, therefore, possible to control their size and distribution by successive treatments after slabbing.

Accordingly, both methods of adding of nitrogen can be used for the same purpose above mentioned.

In this invention, however, the addition of nitrogen from annealing atmosphere is intended to restrict the nitrides formation to the minimum quantity required. The nitrides formed adversely affect the magnetic properties of the final product. The amount of nitrides, therefore, must be limited to minimal and they must be removed after obtaining secondary recrystallization structure.

The denitridification from the 3 percent silicon steel (containing) these nitride forming elements using hydrogen is possible and depends on the content of nitride forming elements and nitrogen, and the thermodynamic properties of the nitrides.

As to Zr, Al and Ta, the nitrides of these elements are less stable than titanium nitride, and consequently the amount of the nitrides of these three elements can be easily decreased by hydrogen reduction after annealing to achieve secondary recrystallization.

The results of the denitridification are shown in Tables 7 and 9. The analysis of the nitrogen in a 3 percent silicon steel is so difficult that a modified Kjeldahl technique was applied, but some uncertainties in the accuracy still remain. As tantalum forms slightly less stable nitride than aluminum, it can easily be removed by denitridification in hydrogen.

It was found that titanium nitride is so stable that the denitridification of the material containing Ti is almost impossible.

Consequently the selection of the nitride forming elements must be made based on the grade of a final product or an end use of the product, and in accordance with the working process.

TABLE 6.—CHEMICAL COMPOSITION OF THE SPECIMEN

|                 |        |
|-----------------|--------|
| No. of specimen | 163    |
| C               | 0.05   |
| Si              | 3.09   |
| Mn              | 0.12   |
| P               | 0.002  |
| S               | 0.001  |
| Zr              | 0.057  |
| $\Sigma N$      | 0.0024 |

secondary recrystallization was carried out for 3 hrs. at 1150° C.

FIG. 3 shows photographs indicating the remarkable effects of nitriding for the secondary recrystallization of the specimens, namely, shows macro-structures after the annealing for secondary recrystallization of each specimen. The photographs of the upper row in FIG. 3 show the macro-structures of the specimens without nitriding namely, those vacuum heated and the photographs of the lower row show macro-structures of the specimens sub-

TABLE 7.—THE RESULTS OF THE DENITRIDING TREATMENTS

| Numbers of specimens | N soluble (percent) | N insoluble (percent) | $\Sigma N$ (percent) | Treatment                                                                            |
|----------------------|---------------------|-----------------------|----------------------|--------------------------------------------------------------------------------------|
| 163-0                | 0.0019              | 0.0005                | 0.0024               | As cold rolled.                                                                      |
| 163-1                | 0.0028              | 0.0010                | 0.0038               | Nitriding for 1 hr. at 700° C. in 18% H <sub>2</sub> plus N <sub>2</sub> atmosphere. |
| 163-2                | 0.0049              | 0.0018                | 0.0067               | Nitriding for 3 hrs. at 700° C. in pure nitrogen.                                    |
| 163-4                | 0.0038              | 0.0010                | 0.0048               | Denitriding for 2 hrs. at 1,150° C. in pure hydrogen.                                |
| 163-5                | 0.0027              | 0.0012                | 0.0039               | Denitriding for 4 hrs. at 1,150° C. in pure hydrogen.                                |
| 163-6                | 0.0037              | 0.0007                | 0.0044               | Denitriding for 8 hrs. at 1,150° C. in pure hydrogen.                                |
| 163-3                | 0.0065              | 0.0005                | 0.0070               | Denitriding for 6 hrs. at 850° C. in pure nitrogen.                                  |
| 163-7                | 0.0040              | Trace                 | 0.0040               | Denitriding for 2 hrs. at 1,150° C. in pure hydrogen.                                |
| 163-8                | 0.0034              | 0.0021                | 0.0055               | Denitriding for 4 hrs. at 1,150° C. in pure hydrogen.                                |
| 163-9                | 0.0037              | 0.0005                | 0.0042               | Denitriding for 8 hrs. at 1,150° C. in pure hydrogen.                                |

TABLE 8.—CHEMICAL COMPOSITION OF THE SPECIMEN

|                 |        |
|-----------------|--------|
| No. of specimen | 160    |
| C               | 0.05   |
| Si              | 3.03   |
| Mn              | 0.11   |
| P               | 0.011  |
| S               | 0.004  |
| Al              | 0.019  |
| $\Sigma N$      | 0.0129 |

jected to nitriding for 5 hours at 750° C. in pure N<sub>2</sub> atmosphere. (No. 156—0.018% Al, No. 160—0.064% Ti, No. 162—0.033% Zr, No. 164—0.11% Zr and No. 166—0.10% Ta).

FIGS. 4 to 6 are photographs which show macrostructure of mono-directional silicon steel sheet obtained under various conditions according to this invention.

The following examples illustrate this invention.

TABLE 9.—THE RESULTS OF THE DENITRIDING TREATMENTS

| Numbers of specimens | N soluble (percent) | N insoluble (percent) | $\Sigma N$ (percent) | Treatment                                              |
|----------------------|---------------------|-----------------------|----------------------|--------------------------------------------------------|
| C-0                  | 0.0112              | 0.0017                | 0.0129               | Nitriding for 10 hrs. at 750° C. in pure nitrogen.     |
| C-1                  | 0.0029              | 0.0020                | 0.0049               | Denitriding for 4 hrs. at 1,000° C. in pure hydrogen.  |
| C-2                  | 0.0012              | 0.0032                | 0.0044               | Denitriding for 4 hrs. at 1,050° C. in pure hydrogen.  |
| C-3                  | 0.0015              | 0.0021                | 0.0036               | Denitriding for 4 hrs. at 1,100° C. in pure hydrogen.  |
| C-4                  | 0.0010              | 0.0020                | 0.0030               | Denitriding for 4 hrs. at 1,150° C. in pure hydrogen.  |
| C-5                  | 0.0008              | 0.0016                | 0.0024               | Denitriding for 4 hrs. at 1,200° C. in pure hydrogen.  |
| C-6                  | 0.0018              | 0.0021                | 0.0039               | Denitriding for 24 hrs. at 1,000° C. in pure hydrogen. |
| C-7                  | 0.0013              | 0.0020                | 0.0033               | Denitriding for 24 hrs. at 1,050° C. in pure hydrogen. |
| C-8                  | 0.0007              | 0.0025                | 0.0032               | Denitriding for 24 hrs. at 1,100° C. in pure hydrogen. |
| C-9                  | 0.0006              | 0.0015                | 0.0021               | Denitriding for 24 hrs. at 1,150° C. in pure hydrogen. |
| C-10                 | 0.0006              | 0.0010                | 0.0016               | Denitriding for 24 hrs. at 1,200° C. in pure hydrogen. |

TABLE 10.—CHEMICAL COMPOSITION OF THE SPECIMEN

|                 |       |
|-----------------|-------|
| No. of specimen | 160   |
| C               | 0.063 |
| Si              | 3.07  |
| Mn              | 0.11  |
| P               | 0.003 |
| S               | 0.004 |
| Al              | 0.006 |
| Ti              | 0.064 |

50 Steels having the chemical compositions as shown in the Table 12 below were prepared and ingots of 100 kg. were produced therefrom. Each ingot was heated at 1000°–1200° C. and then extended into a slab of 100 mm. in thickness x 1 mm. in width x 150 mm. in length by forging. Then said slab was heated to 1250° C. and thereafter hot rolled to a thickness of 2.3 mm. Each hot rolled steel was subjected to pickling, thereafter an-

TABLE 11.—THE RESULTS OF THE NITRIDING OF THE SPECIMEN CONTAINING TITANIUM

| Numbers of specimens | N soluble (percent) | N insoluble (percent) | $\Sigma N$ (percent) | Treatment                                                                            |
|----------------------|---------------------|-----------------------|----------------------|--------------------------------------------------------------------------------------|
| 160-1                | 0.0004              | 0.0013                | 0.0017               | After second cold rolling.                                                           |
| 160-2                | 0.0012              | 0.0017                | 0.0029               | Nitriding for 1 hr. at 700° C. in 18% H <sub>2</sub> plus N <sub>2</sub> atmosphere. |
| 160-3                | 0.0042              | 0.0030                | 0.0063               | Nitriding for 3 hrs. at 700° C. in pure nitrogen.                                    |
| 160-4                | 0.0044              | 0.0019                | 0.0062               | Nitriding for 5 hrs. at 850° C. in pure nitrogen.                                    |

In addition, Table 7, 9 and 11 show the increase of nitrogen content by the nitriding carried out under the various nitriding conditions. The remarkable increase of nitrogen contents can be recognized in every case.

The finely dispersed nitride precipitates formed by nitriding greatly contribute to the secondary recrystallization of these specimens.

In order to distinguish the effect of the fine precipitates from the effect attained without the precipitates, the specimens containing one of each element of Ti, Zr, Ta and Al were heated for 5 hrs. in vacuum or nitrogen atmosphere at 750° C., and then the annealing for sec-

70 nealing (heated at 800° C. for 20 minutes), the first cold rolling (to 0.70 mm. in thickness), decarburization annealing (at 780° C. for 20 minutes), the second cold rolling (to 0.35 mm. in thickness), decarburization annealing (at 780° C. for 20 minutes), then nitriding treatment in an atmosphere as shown below, and thereafter the final annealing. The annealing between the first cold rolling and the second cold rolling is necessary, but the decarburization treatment is not always necessary in the case of steel having a low carbon content,

TABLE 12.—CHEMICAL COMPOSITIONS (WT. PERCENT) OF TESTING MATERIALS

| Sign     | C     | Si   | Mn   | P     | S     | Cu    | Ni    | Cr    | Al    | Ti    | Ta    | Zr    |
|----------|-------|------|------|-------|-------|-------|-------|-------|-------|-------|-------|-------|
| C-----   | 0.05  | 3.03 | 0.11 | 0.011 | 0.004 | 0.082 | 0.06  | 0.04  | 0.019 | ----- | ----- | ----- |
| 126----- | 0.08  | 3.16 | 0.10 | 0.002 | 0.005 | <0.01 | <0.01 | <0.01 | ----- | 0.025 | ----- | ----- |
| 128----- | 0.072 | 3.38 | 0.11 | 0.002 | 0.004 | <0.01 | <0.10 | <0.01 | ----- | ----- | 0.022 | ----- |
| 133----- | 0.08  | 3.13 | 0.18 | 0.004 | 0.006 | 0.02  | 0.01  | <0.01 | 0.006 | 0.21  | ----- | 0.021 |
| 136----- | 0.08  | 3.15 | 0.20 | 0.006 | 0.008 | <0.01 | 0.009 | 0.007 | 0.016 | ----- | ----- | 0.029 |

## EXAMPLE 1

A steel sheet of 0.35 mm. in thickness after the second cold rolling and decarburization treatment, was subjected to nitriding treatment at 500° C. for 10 hours in ammonia gas produced from liquid ammonia and then was cooled to room temperature. Thereafter it was heated in an argon atmosphere from room temperature to 900° C., kept for 2 hours at this temperature, heated to 1150° C., and thereafter was held in a hydrogen atmosphere at 1150° C. for 4 hours. The macro-structure of thus obtained silicon steel sheet is shown in FIG. 4.

## EXAMPLE 2

Each steel sheet of 0.35 mm. in thickness, after the second cold rolling and decarburization treatment was subjected to nitriding treatment at 650° C. for 18 hours in a pure nitrogen gas atmosphere and then was heated to 900° C. in an argon atmosphere, kept 2 hours at this temperature, again heated to 1150° C., and thereafter was held at 1150° C. for 4 hours in a hydrogen atmosphere. The macro-structure of the thus obtained steel sheet is shown in FIG. 5.

## EXAMPLE 3

Each steel sheet of 0.35 mm. in thickness, after the second cold rolling and decarburization treatment, was subjected to nitriding treatment at 750° C. for 4 hours in a pure nitrogen atmosphere and then was heated to 900° C. in an argon atmosphere, kept 2 hours at this temperature, again heated to 1150° C., and thereafter was held at 1150° C. for 4 hours. The macro-structure of thus obtained steel sheet is shown in FIG. 6.

The nitriding atmosphere employed in Examples 2 and 3 may be nitrogen atmosphere containing hydrogen (a mixture gas of less than 15% of hydrogen and balance of nitrogen) which is capable of nitriding the treated steel sheet. Sufficient nitriding effect was seen with such mixture atmosphere but photographs of macro-structure obtained using such atmosphere were not taken.

Regarding Zr containing steel (type 128), a hot rolled sheet of 1.5 mm. in thickness (aside from those mentioned above) was also prepared and was rolled to a sheet of 0.35 mm. in thickness by only one pronounced cold rolling to provide the same result.

The percentages referred to herein are by weight.

What is claimed is:

1. A method of producing a mono-directional silicon steel sheet, comprising the sequential steps of

- selecting a hot and cold rolled silicon steel consisting, aside from incidental impurities, of (a) from 2 to 4% silicon, (b) from 0.01 to 0.10% carbon, and (c) a nitride producing element selected from the group consisting of Al, Ti, Zr and Ta and which when incorporated alone is in the range of 0.01–0.07% Al, 0.01–0.2% Ti, 0.01–0.3% Zr and 0.05–0.5% Ta and when incorporated as two or more elements are within the indicated ranges, the total being however not greater than 0.5%,
- subjecting said hot and cold rolled steel to decarburization treatment,
- nitriding in a nitriding atmosphere the decarburized steel at a temperature of 450° C.–750° C. for 2 to 20 hours to form a finely dispersed nitride precipitate of said element in said steel; and
- subjecting the steel to denitriding treatment at an annealing temperature of between 1,000°–1,200° C. in a hydrogen atmosphere for a time sufficient to remove said nitrides.

2. A method according to claim 1, wherein the nitriding atmosphere is selected from the group consisting of pure nitrogen gas, hydrogen-nitrogen mixture gas and ammonia gas from liquid ammonia.

## References Cited

## UNITED STATES PATENTS

|           |         |                |       |           |
|-----------|---------|----------------|-------|-----------|
| 3,214,303 | 10/1965 | Fiedler        | ----- | 148—111   |
| 3,147,158 | 9/1964  | Fiedler        | ----- | 148—111   |
| 2,802,761 | 8/1957  | Fast           | ----- | 148—113   |
| 3,184,346 | 5/1965  | Fiedler        | ----- | 148—31.55 |
| 3,163,564 | 12/1964 | Taguchi et al. | ----- | 148—111   |
| 3,287,183 | 11/1966 | Taguchi et al. | ----- | 148—111   |
| 3,671,337 | 6/1972  | Kumai et al.   | ----- | 148—113   |
| 2,528,216 | 10/1950 | Dunn et al.    | ----- | 148—16.6  |
| 2,114,802 | 4/1938  | Kinzel         | ----- | 148—16.6  |
| 2,067,896 | 1/1937  | Babinet        | ----- | 148—16.6  |

50 L. DEWAYNE RUTLEDGE, Primary Examiner

W. R. SATTERFIELD, Assistant Examiner

U.S. Cl. X.R.

148—113, 111